

Aug. 13, 1940.

W. J. SCOTT

2,211,170

CERAMIC COATED ARTICLE

Filed Sept. 18, 1937

FIG. 1



FIG. 2



INVENTOR  
W. J. SCOTT

BY *Tommy Robinson*  
ATTORNEY

## UNITED STATES PATENT OFFICE

2,211,170

## CERAMIC COATED ARTICLE

Walter J. Scott, Hinsdale, Ill., assignor to Western  
Electric Company, Incorporated, New York,  
N. Y., a corporation of New York

Application September 18, 1937, Serial No. 164,472

3 Claims. (Cl. 91—73)

This invention relates to methods of making ceramic coated articles and more particularly to methods of making articles having a contrastingly colored coating of vitreous enamel.

5 The present invention is particularly adapted to the production of multi-color or ornamental enamel coatings, such as those used on signs and similar articles. In the usual manufacture of this type of product, variously colored enamels 10 are applied successively to a base and the article is fired after the application of each color. This process has been troublesome because refiring tends to damage the previously fused enamel and thus detract from the utility of the article.

15 An object of this invention is to provide improved methods for producing an article having a protective and durable enamel coating.

In accordance with one embodiment of this invention, an improved process is provided for 20 applying a multi-color enamel coating on a number plate for telephone dials. A ring-shaped base is formed of iron and coated with copper and nickel. A white enamel of suitable composition is prepared for application on the base by pul- 25 verizing, sifting and washing operations to eliminate all particles not included within a predetermined size range. The sized particles or grains of white enamel are fused on the face of the ring and the characters and design are printed thereon with enamel powder of contrasting 30 colors mixed with a suitable vehicle after which the article is refired to mature the characters.

A more complete understanding of the invention may be had by reference to the following 35 description, taken in conjunction with the accompanying drawing, in which

Fig. 1 is a plan view of a number plate embodying the invention, and

Fig. 2 is an enlarged sectional view of the 40 number plate taken on the line 2—2 of Fig. 1.

In producing a number plate in accordance with this invention, a sheet of iron, steel or other suitable material is formed into a ring or base 5. Because only the face of the number plate is 45 covered with enamel, it is desirable to protect the rest of the base against corrosion and this is conveniently accomplished by providing the entire base with an electrodeposited protective coating before the enamel is applied. A preferred coating includes a layer of copper 6 on the iron and a layer of nickel 7 over the copper, which 50 protects the unenameled portion of the base and also bonds satisfactorily with the subsequently applied enamel. If only a copper plating is applied over the iron base, the copper tends to

oxidize and burn off during the fusing of the subsequently applied enamel, while nickel in direct contact with the iron tends to form gases which cause a blistering of the enamel coating. These difficulties are avoided by use of the combination coating and in practice about 20 milligrams of copper per square inch are plated on the base and about 20 milligrams per square inch of nickel are electrodeposited over the copper.

To complete the number plate, a coating of 5 white enamel and identifying characters are applied on the face of the base over the nickel. The white enamel 8 is applied first and used at a suitable temperature. Letters 9, numbers 10, and a 15 background 11 are then applied to the used white enamel in contrasting colors. The characters and markings are formed in ceramic ink, which comprises colored metallic oxides or ceramic enamel particles mixed in a vehicle such as linseed oil. The ink ingredients are mixed to a 20 tacky consistency to prevent running and applied on the enamel surface by means of suitable dies in either a direct or an offset printing process.

The background, which may be blue or black, 25 is applied first and the plate is then placed in an oven and baked at a temperature of about 300° F. to harden the ink so that it will not be marred in subsequent printing operations. The letters, which are usually black, are then printed 30 on the number plate which is then again baked at a temperature of about 300° F. The numerals are usually colored red and are applied in the same manner, after which the entire plate is again fired to fully mature the ceramic ink which 35 requires a temperature around 1300° F. for approximately 4.5 minutes.

In these operations, the repeated firings tend 40 to damage the white enamel applied initially to the base. It is necessary for the white surface to be uniform in color, unblemished and unbroken in the finished product and while these qualities can be provided readily in the enamel as initially fired when the usual materials are employed, refiring tends to cause blistering and "re-boiling" which develops a rough, discolored surface that is unsatisfactory in service. Coating enamels, such as the white enamel used on number plates, are generally applied either in the form of dry powder or by a wet process in which 45 the enamel particles are mixed with water and a flotation agent such as clay. For both of these methods, it has been customary to employ an enamel that is comminuted to a specified maximum particle size. In manufacturing the enam- 50

5

10

15

20

25

30

35

40

45

50

55

el, the pulverizing operation is usually prolonged to eliminate oversize material and this practice produces a variety of particle sizes within the maximum limits. This condition has been considered beneficial, particularly in wet processes where the variety of particle sizes and a high percentage of very fine material promotes uniform distribution of the enamel in the liquid vehicle.

However, it has now been discovered that in processes where refiring of the enamel is necessary, wide variations in particle size is detrimental. It appears that when the usual material is used, interior air pockets are sometimes formed in the enamel body during the initial firing, due, possibly, to early melting of the smaller particles. The surface of the enamel may be unbroken and satisfactory as initially fired, but when the article is heated in the initial stages of refiring, the unequal expansion of enamel and metal causes cracks to form in the weaker spots, that is, through the air pockets. The cracks are filled with air, which may be entrapped as the article becomes hotter, and the surface of the enamel becomes plastic. During the final stage of refiring, the entrapped air expands and causes surface blisters or breaks through to fracture the surface. This action may also force small particles of the undercoating or metal oxide from the base to the enamel surface to impair its appearance and this phenomenon is known as "reboiling." Usually the refiring temperature is insufficiently high or prolonged to cause a final fusing over of the blistered, broken or discolored portions of the surface and these defects therefore remain in the finished product.

These difficulties have been eliminated by the adoption of an enamel which is processed before application to eliminate all particles outside of a predetermined size range. For use on number plates and similar articles, a lead boro-silicate enamel opacified with arsenic oxide is satisfactory for the white coat. In accordance with this disclosure, the enamel is pulverized in a mill and the resultant particles are screened through a 120 sieve. All oversize material is rejected for regrinding and undersized particles are removed from the residue by additional sifting, washing, or by an air separation process.

It is primarily desirable to remove practically all of the fine particles as their presence appears to cause the surface defects on refiring. This can be done conveniently by washing the enamel after the initial sifting. In one satisfactory method, 15 pounds of ground enamel were placed in a 3 gallon jar, the jar filled with water and the supernatant liquid decanted after settling. Before decanting, the jar contained about six times as much water as enamel by volume. It is sometimes necessary to repeat this operation several times to remove all of the undersize material, depending on the particle size distribution, but the operation is readily controlled by observing the progress of the settling period.

The sized particles are applied to the plate

either by sifting or by spraying in a liquid medium containing a flotation agent and fired at 1600° F. for 5½ minutes. The sized particles fire uniformly to produce a homogeneous coating free from air pockets and in the subsequent refiring after application of the character markings the surface of the enamel remains unchanged and no blistering or reboiling occurs. The described materials and processes are suitable for producing all of the qualities desired in a number plate with a single coating of enamel with resultant economies in production costs and the elimination of process defects.

Although the invention has been described in connection with the manufacture of number plates for telephone dials, it will be apparent that it is equally applicable to other ornamented enameled articles and it is understood that the invention is limited only by the scope of the appended claims.

I claim:

1. A method of producing a contrastingly colored enamel coating on a base with an absence of reboiling comprising the steps of applying a finely divided vitreous enamel of specified color on the base and excluding particles that have been eliminated when the enamel is mixed with a relatively larger volume of water and the supernatant liquid is decanted after settling, fusing said enamel on the base, applying a second enamel of contrasting color to portions of the fused enamel, and refiring the base to fuse the second enamel.

2. A method of producing a contrastingly colored enamel coating on a ferrous base with an absence of reboiling comprising the steps of applying a finely divided vitreous enamel on the base, said enamel being in the form of particles sufficiently small to pass through a 120 mesh screen and excluding particles that have been eliminated when the enamel is mixed with about six times its volume of liquid and the supernatant liquid is decanted after settling, fusing said enamel on the base at a specified temperature, applying a second enamel of contrasting color to portions of the fused enamel, and refiring the base at a lower temperature to fuse the second enamel.

3. A method of producing a contrastingly colored enamel coating on a ferrous base with an absence of reboiling comprising the steps of applying a lead boro-silicate enamel on the base, said enamel being in the form of particles sufficiently small to pass through a 120 mesh screen and excluding particles that are eliminated when the enamel is mixed with water in the approximate proportions of one part of enamel to six parts of water by volume and the supernatant water is decanted after a settling period, fusing said enamel on the base at a temperature of 1600° F., applying a mixture of enamel of contrasting color and linseed oil to portions of the fused enamel in the form of characters, and refiring the base at a temperature around 1300° F. to mature the characters.

WALTER J. SCOTT.

CERTIFICATE OF CORRECTION.

Patent No. 2,211,170.

August 13, 1940.

WALTER J. SCOTT.

It is hereby certified that error appears in the printed specification of the above numbered patent requiring correction as follows: Page 1, second column, lines 14 and 16, for the word "used" read --fused--; and that the said Letters Patent should be read with this correction therein that the same may conform to the record of the case in the Patent Office.

Signed and sealed this 5th day of November, A. D. 1940.

(Seal)

Henry Van Arsdale,  
Acting Commissioner of Patents.